

## METHOD FOR THE PREPARATION OF ZINC

James L. Wyatt, South Euclid, Ohio, assignor to  
Horizons Incorporated

No Drawing. Application February 21, 1955  
Serial No. 489,783

8 Claims. (Cl. 75—86)

This invention relates to a process for producing metallic zinc. Metallic zinc is commonly obtained from its ores by two main methods: pyrometallurgical and electrolytic. The pyrometallurgical processes generally depend on the reduction of zinc oxide to the metallic state by carbonaceous reducing gases in retorts, while in the electrolytic process, zinc ores are treated with a suitable acid such as sulphuric acid and the resulting zinc-containing solution is electrolyzed to recover the zinc. My invention is concerned with an improvement in the pyrometallurgical recovery of zinc.

In the recent past the most widely employed process for the pyrometallurgical recovery of zinc was a batch process involving the reduction of a charge of zinciferous material and carbon. Later efforts have been directed toward the development of a continuous process. Possibly the most recent processes evolved in this art are the application of fluidized techniques illustrated in U. S. Patent No. 2,478,912. Each of these prior art processes has been found to be seriously limited in one or more respects. For instance the tendency of impurities usually associated with the zinc-bearing raw material to fuse and agglomerate has constituted the outstanding limitation of most of the pyrometallurgical processes which have been devised. Another problem encountered in the prior art is the reoxidation of the freshly reduced zinc. These and other disadvantages are substantially diminished by the practice of the process constituting the invention herein disclosed.

In accordance with my invention the reduction of a zinc-bearing source material is effected in a molten salt menstruum. By bringing the zinciferous material into contact with a reducing gas in this environment, advantages are obtained which permit the reaction to be effected more rapidly, more efficiently and at lower temperatures than was possible in the prior art processes. In order that the advantages of my process may be better appreciated, a brief description of the present-day methods of producing zinc follows:

(a) *Batch process.*—The present typical batch type process is conducted in a plurality of externally heated clay retorts—6 to 12 inches in diameter and up to 10 feet long. The retorts are open at one end and are positioned with the open end slightly lower than the closed end. They are heated in groups of any desired number by means of gas or oil. They are charged either by hand or by means of a special machine which rams the charge in place. The charge consists of a slightly dampened mixture of zinc oxide and carbonaceous material, usually anthracite coal. The zinc produced by the reduction reaction is condensed and collected as a liquid. The batch usually requires 24 to 48 hours from charge to charge. The process has always been recognized as burdened with high labor costs, poor heat transfer, slow reaction rates, waste of the carbon monoxide produced, loss of zinc by reoxidation to zinc oxide, nonuniformity of the product and low yield. As a result a number of continuous processes have been suggested.

(b) *Continuous processes.*—The above described batch process led to the development of a continuous vertical retort process, described in detail in volume 121 of the Transactions of the A. I. M. E. beginning on page 427. Briefly, a charge mixture consisting of oxide ore or roasted concentrate, binder and carbonaceous reducing material is briquetted. The briquettes are dried and then coked and are charged, preferably hot as they leave the coking furnace, into the upper portion of a vertical heating chamber wherein they are heated to complete the reduction of the zinc. The metal and gases produced during the reaction pass upwardly to a condenser and the spent briquettes pass downwardly to a point of discharge. The process requires elaborate equipment and special precautions are required to prevent the freshly reduced zinc from condensing within the furnace or re-oxidizing to form blue powder.

(c) *Fluidized continuous process.*—As previously noted a more recently developed continuous process involves the fluo-solids technique. Thus, in Patent No. 2,478,912 a process is described in which comminuted reducible zinc compounds may be reduced by either a solid or a gaseous reducing agent by introducing the zinc compound into a reducing zone consisting predominantly of a suspension of particles of a solid diluent in a gas. The zinc formed by reduction passes continuously out of the reaction vessel and is condensed. In the aforesaid patented process the comminuted zinc compound is supplied in finely divided form to a reducing zone, along with the solid diluent. A fluidizing gas is admitted to the lower portion of the reducing zone to maintain the solid diluent and zinc-containing material in a fluidized condition. The entire fluidized bed is heated by suitable means to temperatures between 1600° and 2300° F., at which temperatures the zinc compound is readily reduced by carbon or carbon monoxide to form zinc vapor which passes off along with carbon monoxide.

(d) *The present invention.*—In accordance with my invention a comminuted zinc compound is reduced by carbon monoxide in a fused bath which may advantageously contain carbon in finely divided form. The resulting zinc vapor is continuously withdrawn and condensed by suitable means. By continuously feeding the several reactants into the fused bath and by continuously withdrawing the products from the system, the entire process can be carried out in a manner which is free from the obvious disadvantages of the batch type processes described above.

Another advantage possessed by my process, particularly when compared with either of the continuous processes described above lies in the simplicity of the apparatus required as compared with the highly specialized apparatus employed in the prior art processes. Other advantages will become apparent from the following description.

The most significant departure from the prior art resides in the use of a fused bath as the environment for carrying out the reduction of a reducible zinc compound. The materials chosen for the fused bath must have a melting point below the temperature at which the reduction takes place and at the same time must possess a vapor pressure which is very low at the reaction temperatures. In addition, in many instances, it may be found desirable to choose as one or more of the components of the fused bath material which fluxes the anticipated impurities in the zinciferous raw material to be reduced. I have found that the alkali metal chlorides are particularly suited to carrying out my process. Sodium chloride or mixtures of sodium chloride and potassium chloride have been found to possess the desirable combination of properties and to be readily adapted to the execution of my process. By employing

a fused bath as the reaction environment, previous disadvantages of the prior art resulting from the tendency of the charges to fuse or agglomerate are completely avoided.

The comminuted zinc compound fed into the fused salt bath may comprise either a raw zinc ore or a beneficiated zinc ore. In the event that the latter is available, for instance, in the form of a roasted concentrate, it is reduced to a finely divided powder by any suitable means in order to expedite the desired reduction reaction.

The reduction reaction is effected in the fused bath by means of a reducing gas which is sparged into the bath in very finely divided form. Any suitable reducing gas may be employed and carbon monoxide containing mixtures have been found to be particularly effective. The reducing gas tends to dissolve in the fused salt bath and accordingly there is obtained a reaction between gas dissolved and the solid to be reduced in addition to a reaction between the gas itself and the solid to be reduced.

In order that reducing conditions may be insured in the system, it has been found expedient to include additional carbon in the bath in finely divided form. The carbon particles are continuously agitated by the gas introduced into the melt and thus are continuously brought into contact with fresh material such as carbon dioxide formed by reduction of the zinc oxide, which the particles reduce to reform carbon monoxide.

As a result of the reaction, zinc vapor and other gaseous products are continuously evolved from the bath and are withdrawn therefrom. The temperature of the reaction is chosen so that the zinc will have an appreciable vapor pressure and hence, it is possible to operate at temperatures below the boiling point of zinc (1706° F.) and at temperatures below those conventionally employed in this art. For example, in accordance with my invention the reduction is effected at temperatures between about 1400° F. and 1550° F. or higher. The zinc vapor and other gases are passed into a condenser and by control of the condenser temperature, the zinc may be obtained either in the form of a liquid or in the form of a finely divided solid. The following specific example will serve to further illustrate the advantages of my invention:

#### Example

A mixture was prepared by thoroughly mixing 162 parts by weight of zinc oxide, 30 parts by weight of carbon and 850 parts by weight of sodium chloride. The mixture was charged into a reaction furnace provided with heating means and heated to a temperature of approximately 850° C. (1562° F.). After the salt had melted, carbon monoxide was introduced through a porous tube, so that the gas was distributed throughout the melt. The furnace was provided with a cover having an offtake to permit withdrawal of gaseous products. The gases evolved were passed through a condenser constructed of graphite, from which a bright metallic product of elemental zinc was recovered. While the above process was run as a batch process, it could be readily converted to a continuous process.

From the above it will be seen that my process is characterized by a number of advantages. Firstly it will be noted that the apparatus required is simple in nature. Essentially the only major units of equipment necessary comprise: a means to produce a suitable reducing gas such as water gas, producer gas, or pure carbon monoxide; a reducing furnace and a condenser. If a reducible zinc compound is not available in comminuted form obviously means must be furnished for obtaining this material. Such means could include a furnace in which zinc sulfides or other zinc compounds are converted to zinc oxide and crushing means for pulverizing the oxide product. Optionally, in the event that the zinc is collected in molten form a means for casting the zinc may be provided.

I claim:

1. A process for the reduction of a reducible zinc compound which comprises establishing a fused bath of at least one alkali metal chloride salt, introducing a zinc compound and a reducing agent into the fused bath, effecting reduction of the zinc compound in said fused bath at a temperature below the boiling point of zinc metal, recovering zinc from the gaseous effluent from said fused salt bath.
- 5 2. A process for producing metallic zinc which includes forming a fused bath consisting essentially of at least one alkali metal chloride, introducing a reducible zinc compound and a gaseous reducing agent into the fused alkali metal chloride bath, maintaining the bath at a temperature at which zinc metal has an appreciable vapor pressure and thereby effecting the reduction of the zinc compound and recovering the zinc so produced from the gaseous effluent from said fused bath.
- 10 3. A process for producing metallic zinc including forming a fused bath consisting essentially of at least one alkali metal chloride, introducing a reducible zinc compound and a carbon monoxide containing reducing gas into the fused bath, maintaining the fused bath at a temperature of at least about 1400° F., and recovering the zinc so-produced from the gaseous effluent from said fused bath.
- 15 4. A process for producing metallic zinc including forming a fused bath consisting essentially of at least one alkali metal chloride, a reducible zinc compound and finely divided carbon, and introducing a carbon monoxide containing reducing gas into the fused bath, maintaining the fused bath at a temperature of between about 1400° F. and 1550° F., and recovering the zinc so-produced from the gaseous effluent from said fused bath.
- 20 5. A process for producing metallic zinc including forming a fused bath comprising sodium chloride, introducing a reducible zinc compound and a carbon monoxide containing reducing gas into the fused bath, maintaining the fused bath at a temperature of at least about 1400° F., and recovering the zinc so-produced from the gaseous effluent from said fused bath.
- 25 6. A process for producing metallic zinc including forming a fused bath consisting essentially of at least one alkali metal chloride and solid finely divided carbon, introducing zinc oxide and a carbon monoxide containing reducing gas into the fused bath, maintaining the fused bath at a temperature of between about 1400° F. and 1550° F., and recovering the zinc so-produced from the gaseous effluent from said fused bath.
- 30 7. A process for producing metallic zinc including forming a fused bath essentially comprising sodium chloride, introducing zinc oxide and a reducing gas into the fused bath, maintaining the fused bath at a temperature of at least about 1400° F. but not exceeding about 1706° F., and recovering the zinc so-produced from the gaseous effluent from said fused bath.
- 35 8. A process for producing metallic zinc including forming a fused bath comprising sodium chloride, introducing zinc oxide and carbon monoxide gas into the fused bath, maintaining the fused bath at a temperature of between 1400° F. and 1550° F., and recovering the zinc so-produced from the gaseous effluent from said fused bath.
- 40 9. A process for producing metallic zinc including forming a fused bath comprising sodium chloride, introducing zinc oxide and a carbon monoxide containing reducing gas into the fused bath, maintaining the fused bath at a temperature of at least about 1400° F., and recovering the zinc so-produced from the gaseous effluent from said fused bath.
- 45 10. A process for producing metallic zinc including forming a fused bath comprising sodium chloride, introducing zinc oxide and a carbon monoxide containing reducing gas into the fused bath, maintaining the fused bath at a temperature of between about 1400° F. and 1550° F., and recovering the zinc so-produced from the gaseous effluent from said fused bath.
- 50 11. A process for producing metallic zinc including forming a fused bath comprising sodium chloride, introducing zinc oxide and a carbon monoxide containing reducing gas into the fused bath, maintaining the fused bath at a temperature of between about 1400° F. and 1550° F., and recovering the zinc so-produced from the gaseous effluent from said fused bath.
- 55 12. A process for producing metallic zinc including forming a fused bath comprising sodium chloride, introducing zinc oxide and a carbon monoxide containing reducing gas into the fused bath, maintaining the fused bath at a temperature of between about 1400° F. and 1550° F., and recovering the zinc so-produced from the gaseous effluent from said fused bath.
- 60 13. A process for producing metallic zinc including forming a fused bath comprising sodium chloride, introducing zinc oxide and carbon monoxide gas into the fused bath, maintaining the fused bath at a temperature of between 1400° F. and 1550° F., and recovering the zinc so-produced from the gaseous effluent from said fused bath.
- 65 14. A process for producing metallic zinc including forming a fused bath comprising sodium chloride, introducing zinc oxide and a carbon monoxide containing reducing gas into the fused bath, maintaining the fused bath at a temperature of between about 1400° F. and 1550° F., and recovering the zinc so-produced from the gaseous effluent from said fused bath.

#### References Cited in the file of this patent

#### UNITED STATES PATENTS

|    |           |                |               |
|----|-----------|----------------|---------------|
| 70 | 37,803    | Bennett        | Mar. 3, 1863  |
|    | 681,609   | De Bechi       | Aug. 27, 1901 |
|    | 1,431,877 | Diehl          | Oct. 10, 1922 |
|    | 1,913,929 | Kerschbaum     | June 13, 1933 |
|    | 2,382,565 | Hedberg        | Aug. 14, 1945 |
|    | 2,685,506 | Schereschewsky | Aug. 3, 1954  |
|    | 2,701,194 | Deterding      | Feb. 1, 1955  |
| 75 | 2,745,736 | Loevenstein    | May 15, 1956  |